

# UNITED STATES PATENT OFFICE.

GUSTAV SPITZ, OF BRÜNN, AUSTRIA-HUNGARY, ASSIGNOR TO GOLDSCHMIDT DETINNING COMPANY, OF NEW YORK, N. Y., A CORPORATION OF NEW JERSEY.

## PROCESS OF OBTAINING METALS, &c., SOLUBLE IN ALKALIS.

1,129,431.

Specification of Letters Patent.

Patented Feb. 23, 1915.

No Drawing.

Application filed April 21, 1908. Serial No. 428,438.

*To all whom it may concern:*

Be it known that I, GUSTAV SPITZ, manager, a citizen of Austria-Hungary, residing at Brünn, Moravia, Austria-Hungary, have invented a Process of Obtaining Metals, &c., Soluble in Alkalies; and I do hereby declare the following to be a full, clear, and exact description of the same.

My invention relates to a process for separating valuable metals, or their salts, from their compounds, mixtures and alloys.

It relates particularly to a process of obtaining from metallic mixtures, compounds or alloys their alkaline compounds directly, and then treating the resulting alkaline compounds to obtain the pure metals or valuable compounds of the same.

The process is particularly adapted for removing from their impure compounds or mixtures the following metals: tin, zinc, lead, copper, iron, antimony, bismuth, silver, nickel, cobalt and residue thereof. From these materials their alkaline compounds can be procured directly, for example from impure tin, stannate of soda (a salt used in color preparation); from this solution, by precipitation with acids (for example  $\text{CO}_2$ ,  $\text{SO}_2$ ,  $\text{NaHCO}_3$ ) I may obtain tin oxide; from this tin oxide, by solution in  $\text{HCl}$ ,  $\text{SnCl}_4$  and  $\text{SnCl}_2$ , by reduction with carbon, pure tin. As alkaline solutions I preferably employ caustic soda or sulfid of sodium, or other similar acting reagents. To the alkaline solutions thus obtained, I add oxidizing agents, such as saltpeter, dioxid of manganese or potassium chromate, and then obtain from the oxidized solution the metal or metallic compound. This may be done by evaporating the solution after the impurities have been removed, or the metallic oxides may be precipitated by an acid, and the pure metal obtained by reduction or electrolytically.

The amount and concentration of the alkaline solution depend upon the metal, or compound to be treated. The concentration must be such as to allow the metallic compound produced to be completely dissolved.

Assume that it is required to heat a mixture or compound or an impure metal con-

taining tin, zinc, lead, iron and copper. The chemical formulæ are the following:



The iron and copper are not dissolved, but remain, perhaps as a lower oxid, in the slimes. In order to nullify the action of the hydrogen, and assist the operation, oxidizing materials are now added.

Taking tin as an example, the reaction is shown by the following formulæ: 65



Using saltpeter:



The solution employed in treating the metal-containing substance or substances should have a temperature of  $100^\circ \text{ C}$ . or over, and the pressure should be from 7 to 15 atmospheres. This is an essential feature of my invention.

At the completion of the operation, there is obtained tin, zinc, and lead in solution as the corresponding sodium compounds. 80 Iron and copper are dissolved as slime. Zinc and lead are removed from the solution, for example, by means of sodium sulfite, and the tin, as stated above, either as such, or in any form of combination free from other heavy metals. The iron and copper and any stray particles of the other metals may be recovered from the slime, by means of the proper reagent.

Having thus fully described my improved 90 process, what I claim is:—

1. A process of obtaining valuable metals or metallic compounds soluble in alkalies from metal-containing substances, which consists in subjecting such a substance to 95 the action of an alkaline solution at super-atmospheric pressure, and then treating the resulting solution to obtain the valuable metals or compounds.

2. A process of obtaining valuable metals 100 or metallic compounds soluble in alkalies from metal-containing substances, which

consists in subjecting such a substance to the action of an alkaline solution at a pressure of 7 to 15 atmospheres, and then treating the resulting solution to obtain the valuable metals or compounds.

3. A process of obtaining valuable metals or metallic compounds soluble in alkalis from metal-containing substances, which consists in subjecting such a substance to 10 the action of an alkaline solution at a super-atmospheric pressure and temperature of over 100° C., and then treating the resulting solution to obtain the valuable metals or compounds.

15 4. A process of obtaining valuable metals or metallic compounds soluble in alkalis from metal-containing substances, which consists in subjecting such a substance to the action of a hot alkaline solution at a 20 pressure of 7 to 15 atmospheres, and then treating the resulting solution to obtain the valuable metals or compounds.

25 5. A process of obtaining valuable metals or metallic compounds soluble in alkalis from metal-containing substances, which consists in subjecting such a substance to the action of an alkaline solution having a temperature of over 100° C. at a pressure of 7 to 15 atmospheres, and then treating

the resulting solution to obtain the valuable 30 metals or compounds.

6. A process of obtaining valuable metals or metallic compounds soluble in alkalis from metal-containing substances, which consists in subjecting such a substance in 35 the presence of an oxidizing material to the action of an alkaline solution at a pressure of 7 to 15 atmospheres, and then treating the resulting solution to obtain the valuable metals or compounds.

7. A process of obtaining valuable metals or metallic compounds soluble in alkalis from metal-containing substances, which consists in subjecting such a substance in the presence of an oxidizing material to the 40 action of an alkaline solution having a temperature of over 100° C. at a pressure of 7 to 15 atmospheres, and then treating the resulting solution to obtain the valuable metals or compounds.

50 In testimony whereof, I have signed my name to this specification in the presence of two subscribing witnesses.

GUSTAV SPITZ.

Witnesses:

MORITZ SCHMOLKAY,  
LEOPOLD DRDÁCVIJ.